

April 21, 1925.

1,534,738

C. H. ROE

METHOD OF DRYING VARNISH

Filed March 31, 1920



Fig. 1



Fig. 2

Charles H. Roe.  
By his Attorneys  
Blackmore, Spencer & Flint.

Inventor

## UNITED STATES PATENT OFFICE.

CHARLES H. ROE, OF TARRYTOWN, NEW YORK, ASSIGNOR TO GENERAL MOTORS CORPORATION, OF DETROIT, MICHIGAN, A CORPORATION OF DELAWARE.

## METHOD OF DRYING VARNISH.

Application filed March 31, 1920. Serial No. 370,278.

To all whom it may concern:

Be it known that I, CHARLES H. ROE, a citizen of the United States, and a resident of Tarrytown, county of Westchester, and 5 State of New York, have invented certain new and useful Improvements in Methods of Drying Varnish, of which the following is a full, clear, concise, and exact description, such as will enable others skilled in the 10 art to which the invention relates to make and use the same.

My invention relates to the art of coating articles with varnish, japan, enamel, paint or like protective coating material, and particularly to the drying and hardening of a film of coating material applied to the articles in the liquid form; and the character of which material is such that the articles being coated have to be heated to a comparatively high temperature in order to secure the drying and oxidation of the film, and a satisfactory finished coating for the article.

The object of my invention is to provide an improved method or process for accomplishing the drying and hardening of a film of liquid coating composition applied to the articles and by the use of which process a better adhering, a more durable, a better appearing and an otherwise more satisfactory coating and protection for the articles will be secured; my invention being particularly adapted for use in the enameling or varnishing of metallic sheet metal parts used in the construction of bodies for automobiles.

35 Varnishes, japans, paints and like liquid coating compositions used for the coating of metal articles such, for example, as the various metal parts of the body of an automobile, may be defined generally as composed of a suitable liquid vehicle in which suitable gums and resins, together with pigments which determine the color of the coating, are dissolved and held in suspension; the liquid vehicle being composed in part of a

40 drying oil which is oxidized during the setting and hardening of the coating film and in part of a volatile solvent or material employed for the purpose of thinning the liquid coating composition so that the same 45 may be the more readily applied to the article or surface to be coated; and which solvent or thinning liquid must be driven off from the film of coating material before the same can become dry and hard as the 50 same has no drying qualities as that term

is used in the varnishing, painting and generally in the coating art.

Ordinary linseed oil may be cited as perhaps the best known example of a liquid vehicle which will oxidize under conditions 60 such that a free supply of air has access thereto and in which the gums, resins, color materials, driers and other substances are dissolved and held in suspension; while the volatile solvent or thinning material, which 65 commonly has no drying or oxidizable properties, may be a petroleum product such as gasolene, benzine, alcohol, or in fact any easily volatile liquid which will mix with the more viscous drying oil and gums which, 70 particularly in the case of japans, is so thick as to render the application thereof to articles to be coated difficult unless a thinning liquid is first mixed therewith.

The film of coating material applied in the 75 liquid form to the article to be coated must obviously become dry and hard before the film becomes fixed upon the surface to which it is applied and assumes the character of a permanent and strongly adherent coating 80 necessary in actual practice.

The ultimate drying and hardening of an initial film of liquid coating composition involves two steps or operations which are for the most part essentially separate and distinct from one another, although the end of the first or drying step proper in a sense merges with the beginning of the second or hardening step; the first of said steps involving the evaporation or the driving off 85 therefrom of the volatile solvent or thinning ingredient of the coating film, while the second of said steps is characterized by the absorption of oxygen from a surrounding body of air which accomplishes the oxidation and 90 hardening of the linseed or equivalent drying oil ingredient which enters into the composition of the coating film.

Heretofore to the best of my knowledge and belief no attempt has been made to separate 100 the two phases above referred to through which the liquid coating film passes in attaining its final form of a dry, hard, resistant, and strongly adhering coating or finish upon the article or surface to be protected; although said phases are essentially 105 separate and distinct from one another and involve entirely different processes, the first being a purely physical and the second an essentially chemical process. After the 110

japan, varnish or paint has been applied to the articles they have heretofore commonly been passed into an oven or enclosure heated to a comparatively high temperature, and left therein for a time which experience dictated as that proper to secure a dry and sufficiently hard coating upon the surface or article being treated; all as a single and uninterrupted process or operation.

10 It will be appreciated that while the volatile solvent constituent of the liquid coating film must be completely eliminated before the resultant coating will be of sufficient hardness to afford the requisite degree of 15 protection to the article, even though the drying oils and gums thereof may ultimately become completely oxidized, there is no necessary connection between the primary volatile liquid driving off step and the subsequent oxidizing step of the entire drying 20 and hardening process regarded as starting with the freshly applied film of liquid coating material, and ending with the dry and hard layer of protecting material secured in 25 varnishing processes.

In my improved varnish drying process (by which term I mean all the steps involved in the conversion of a freshly applied film of liquid coating composition into a finished oxidized, dry, hard, and resistant protecting layer or coating, as distinguished from the "drying" which involves the final oxidation of the drying oil ingredient of the composition) the first step or phase which 30 involves the evaporation of the volatile solvent or thinning liquid ingredient of the film is isolated from the second step or phase which involves the absorption of oxygen from atmospheric air by the drying oil constituent of the varnish and the hardening 35 or oxidation of the said film.

Inasmuch as the evaporation of the volatile solvent constituent of the liquid coating film is commonly accomplished under 45 conditions such that the articles being coated are surrounded by a gaseous medium containing oxygen, and under conditions such that there will be a simultaneous oxidation of the drying oil constituent of the film; and in order that the resulting finished layer 50 of varnish material may be roughened as little as possible by minute bubbles of the volatile constituent breaking through a surface of the film which has taken up some oxygen from the gaseous medium and has begun to harden; I preferably drive off the volatile liquid ingredient as rapidly as possible during the first phase or step of my improved drying process in order that the 55 complete or substantial elimination of such liquid may be accomplished before the drying oil constituent has had time to become oxidized to any material degree, and before a surface layer has been formed which

would be broken or roughened by the escape 65 of volatile material from the inner portions of the film from which the volatile ingredient is being eliminated. The subsequent or second phase of the process during which the drying oil and gums become oxidized 70 by the absorption of oxygen from a surrounding gaseous medium and a finished coating is secured is then permitted to proceed more slowly, thus increasing the hardness, the adherent property, and the general 75 excellence of the resulting finished layer of coating material upon the article being treated.

The first or primary stage of my improved varnish drying process during which the volatile solvent material of the film is eliminated is obviously in no way dependent upon the presence of oxygen in the gaseous medium surrounding the articles and through which heat is commonly communicated thereto, to accomplish the vaporization of the volatile products, whereas the subsequent or secondary stage of the process during which the oxidation of the coating remaining upon the articles is accomplished necessitates the presence of oxygen in such gaseous medium; and such final stage proceeds the more rapidly, and is the more satisfactory and complete, the greater the amount of oxygen present in the gaseous 90 medium from which the oxygen is derived. For these reasons my process is the better carried out by heating the articles being coated to a comparatively high temperature in a closed chamber containing a gaseous 95 medium, such as air, which, however, is quiescent, except for unavoidable currents due to convection, that is, in a chamber to which no fresh air is purposely supplied during the primary or volatile liquid evaporating stage; and by supplying air in abundance, and at a much lower temperature, to the space surrounding the articles during the secondary or oxidizing stage of the process. Such a method of procedure secures an effective and efficient application of heat to the article during the volatile liquid eliminating stage and reduces the heat required to drive off the volatile products during the first or primary stage of 110 the process; and at the same time provides oxygen in abundance, and even in excess, during the secondary or oxidizing stage, so that the oxidation of the drying oil and gums may proceed rapidly and effectively. 115

Although the process wherein my invention consists may be performed by various forms of apparatus or device, I have in the accompanying drawing illustrated one form of apparatus capable of performing the 120 same, and which I have found to be satisfactory for that purpose. In said drawing; Figure 1 is a perspective view broken

away in part showing an apparatus suitable for performing the first of the two steps wherein my invention consists; and

5 Figure 2 is a sectional view illustrating an apparatus or device capable of use in performing the second step of my improved process.

In performing my improved process the essential steps of which have been herein-  
10 before enumerated the articles being treated are first coated with japan, varnish, paint or equivalent liquid coating material in any way, as by dipping them in a bath of such material, by spraying the same thereupon, 15 by means of a brush, or otherwise; after which the said articles are placed within a closed chamber such, for example, as the chamber or oven 1, Figure 1, having a heating coil 2, and an outlet flue 3 through which 20 such gases as may be produced may pass off and heated to a temperature, and for a period sufficient to vaporize the volatile solvent or thinning constituent of the film of coating material. It is preferable that there be 25 no supply of fresh air to the heating chamber during this first or evaporating stage of the process, as the oxidation of the film should be as far as possible prevented during this phase of the process; and the tem- 30 perature should be high in order to accomplish the vaporization of the volatile products quickly, and reduce the time during which some slight and unavoidable oxidation 35 of the film may occur.

The evaporating step of the process may be hastened by heating the articles in a chamber in which a reduced pressure is maintained by means of a vacuum producing pump or equivalent device; and the oxidation which to a degree is unavoidable during the first stage of the process may be reduced by heating in an atmosphere having a reduced oxygen content, should such refinement in the process be deemed desirable and of sufficient practical importance to justify the somewhat greater difficulty and expense incident to the performance thereof under reduced pressure, and in a gaseous medium in which the oxygen is reduced in quantity. The heating of an unchanging mass of air or equivalent gaseous medium may obviously be the more efficiently accomplished than would be the case if fresh air was supplied to the heating chamber during the first or driving off stage of the process during which the volatile constituents of the film of liquid coating material are eliminated.

60 After the volatile solvent ingredient has been completely or sufficiently eliminated from the film of liquid coating material an abundant supply of oxygen is supplied to the article being coated, so that the oxida-

tion and hardening of the residual portion of the film will take place. This second step of my process is preferably performed in a separate chamber such, for example, as the chamber 4, Figure 2, to which the articles are transferred and through which chamber an abundant supply of air is caused to flow as by means of a fan blower 5 which discharges thereinto through the conduit 6, or other type of air forcing means, the temperature of such stream of air being usually materially lower than the temperature to which the articles were subjected during the first or evaporating stage of the process, although such air will ordinarily be heated to a comparatively moderate degree as by the heating coil 7; as the important consideration during this second stage or phase of the process is to provide an abundant supply of oxygen so that the oxidation of the drying oil will occur with rapidity and efficiency, rather than a high temperature as no volatile constituents of the film remain to be eliminated; such constituents having been eliminated during the first stage of the process.

As a matter of course the temperature employed during the primary and secondary stages of my process, the duration of such stages, and other purely manipulative steps may be varied within wide limits without in any way departing from my invention the essential steps of which are the primary step or stage during which the volatile products are eliminated, followed by the secondary stage or step during which oxidation of the drying oil present in the film is accomplished; the two steps or phases being separated from one another and each limited, so far as is practicable, to the particular end to be attained during such stage. In the practical operation of my process upon metallic body members, fenders therefor, hood structures, and like sheet metal automobile body parts I have secured satisfactory results by first dipping said articles in a bath of japan or equivalent varnish; then permitting excess varnish to drain from said members and flow back into the tank containing the bath; then transferring said articles to an oven or chamber which, so far as feasible is closed, and to which there is no designed supply of fresh air; then heating said articles within the chamber aforesaid to a temperature of approximately 500 degrees Farenheit, for a period of approximately ten minutes; then transferring said articles to a second chamber through which an abundant flow of clean fresh air heated to a temperature of approximately 250 degrees Farenheit is maintained; the articles being permitted to remain in the second chamber until the oxidation of the coating

is completely accomplished and until a satisfactory, hard, and properly adherent coating is secured.

Among the advantages secured in the drying of a film of varnish, japan, or equivalent liquid coating composition in accordance with my invention are increased efficiency as regards the consumption of heat during the drying process, because the heating is done in an oven or chamber in which an unchanging mass of air is maintained thus avoiding the waste incident to the heating of a large volume of air to the high temperature necessary to accomplish the vaporization of the volatile constituents of the film; as no flow of air heated to the temperature necessary to vaporize such products is maintained past the articles throughout the drying of the film or for a considerable part of the drying process. The heating of the articles to a high temperature and in a quiescent body of air during the evaporating stage of the process reduces surface oxidation to a minimum during such first stage and secures the elimination of the volatile constituents of the film before any material oxidation thereof can take place; so that the partially dried and hardened layer is not broken or disturbed by the escape of volatile constituents after such first step and during the oxidizing phase; because the volatile products have already been eliminated and because the articles are heated to a much lower temperature during the second stage of the process; from which it follows that a smooth surface is secured in the resulting layer or varnish at the end of the process. Furthermore, the carrying out of the oxidizing step of the process by means of a large volume of air heated to a moderate temperature, or in fact at atmospheric temperature in many cases, results in a more completely oxidized and in a harder and more satisfactory, and a better appearing coating upon the articles being coated.

Having thus described and explained the process wherein my invention consists, I claim and desire to secure by Letters Patent:

1. The method of drying a liquid coating composition containing a volatile ingredient and a drying oil applied as a film to an article to be coated which consists in heating the article to thereby evaporate the volatile constituent of said film as a first step or phase; and oxidizing the remaining portion of said film as a second step or phase separate and distinct from said first mentioned evaporating stage.

2. The method of drying a liquid coating composition containing a volatile ingredient and a drying oil applied as a film to an article to be coated which consists in heating the article to a comparatively high temperature, and for a comparatively short time, to thereby rapidly drive off the volatile constituent of said film therefrom as a first step or phase; and heating the article being coated to a materially lower temperature, and for a comparatively long time, to thereby accomplish the oxidation of the drying oil constituent of said film as a step or phase separate and distinct from said first mentioned stage.

3. The method of drying a liquid coating composition containing a volatile ingredient and a drying oil applied as a film to an article to be coated which consists in heating the article within a chamber in which a limited amount of oxygen is present, to thereby evaporate the volatile constituent from said film, as a first step or phase; and then oxidizing the drying oil constituent of said film in a chamber wherein an abundant supply of oxygen is present as a second step or phase separate and distinct from said first mentioned phase.

4. The method of drying a liquid coating composition containing a volatile ingredient and a drying oil applied as a film to the article to be coated which consists in heating the article being coated to a comparatively high temperature, and for a comparatively short time, within a chamber containing a quiescent body of gaseous medium, to thereby drive off the volatile constituent of said film as a first step or phase; and then subjecting the article being coated to the action of a comparatively large volume of air to thereby oxidize the remaining portion of said film as a second step separate and distinct from said first mentioned step.

5. The method of drying a liquid coating composition containing a volatile ingredient and a drying oil applied as a film to an article to be coated which consists in heating the article in a chamber containing a limited quantity of air to a high temperature, and for a comparatively short time, to thereby rapidly evaporate the volatile constituent of said film as a first step or phase; and then causing a stream of air heated to a moderate temperature to flow past the article being coated to thereby oxidize the remaining portion of the film as a second step or phase separate and distinct from said first mentioned phase.

In testimony whereof I affix my signature.  
CHARLES H. ROE.